

Dec. 25, 1962

N. J. GRANT

3,070,468

METHOD OF PRODUCING DISPERSION HARDENED TITANIUM ALLOYS

Filed Oct. 29, 1958

FIG. 3



FIG. 4



FIG. 2



FIG. 1



INVENTOR  
NICHOLAS J. GRANT  
BY  
*E.J. Kallil*  
ATTORNEY

## 1

3,070,468

## METHOD OF PRODUCING DISPERSION

## HARDENED TITANIUM ALLOYS

Nicholas J. Grant, 10 Leslie Road, Winchester, Mass.  
Filed Oct. 29, 1958, Ser. No. 770,392

13 Claims. (Cl. 148—20.3)

This invention relates to dispersion-hardened titanium group metals and alloys based on these metals and in particular to a method for producing a titanium-base alloy characterized by high strength at elevated temperature, such as improved resistance to creep.

In recent years, titanium and zirconium have achieved some measure of prominence as new engineering materials. They have high melting points (about 3200° F. and 3350° F., respectively) which would appear to adapt them for use as a load carrying structural element at elevated temperatures. Unfortunately, this is not the case as wrought titanium and zirconium are characterized by low resistance to creep at relatively high temperatures.

With respect to titanium, it is subject to instability when used over certain temperature ranges arising from the transformation of beta to alpha or intermediate phase products, whereby the physical properties are adversely affected. The alpha phase, which comprises an hexagonal-close-packed structure, is the desirable structure propertywise. The beta phase, which is body-centered-cubic structure, has lower strength properties and, therefore, is less desirable. Hence, the addition of alloying elements which tend to promote the formation of the beta structure is avoided as far as it is possible while those which tend to stabilize the alpha phase are preferred. However, only a few elements, such as aluminum or tin, are alpha stabilizers. Any method for strengthening titanium and titanium-base alloys without relying on phase stabilization or transformation would be desirable, particularly any method which would increase the load carrying power up to 1200° F.

I have discovered a method whereby the high temperature strength properties of titanium group metals (i.e. Ti, Zr and Hf), particularly titanium and its alloys, can be greatly improved by utilizing the principle of dispersion hardening. The hardening and strengthening of these metals are achieved by relying on their propensity to absorb oxygen in solid solution. Titanium in particular has a high affinity and solubility for oxygen (about 15% by weight oxygen) which normally has a deleterious effect on its properties. My discovery resides in producing a titanium-base alloy containing a small amount of a rare earth metal in solid solution therewith, which alloy is hardened by subsequent treatment under controlled oxidizing conditions to convert the rare earth metal to finely dispersed refractory oxide.

It is the object of this invention to provide a method for dispersion hardening titanium group metals and their alloys, in particular titanium and titanium-base alloys.

It is also an object to provide a dispersion hardened wrought compositon of titanium group metals and their alloys.

Another object is to provide as an article of manufacture a titanium or titanium alloy composition characterized by improved strength properties at elevated temperatures.

These and other objects will more clearly appear from the following disclosure and the accompanying drawing, wherein:

FIG. 1 is an equilibrium diagram of the titanium-rich binary showing the various phases that exist for cerium contents ranging up to about 6%.

FIG. 2 is an equilibrium diagram of the titanium-rich portion of the titanium-lanthanum binary showing the

## 2

various phases that exist for lanthanum contents ranging up to about 6%.

FIG. 3 is a representation of a photomicrograph taken at 2500 times magnification showing a dispersion of  $\text{CeO}_2$  in an equiaxed alpha matrix of titanium after internally oxidizing a titanium alloy containing 0.7% Ce; and

FIG. 4 is a representation of a photomicrograph at 2500 times magnification of an internally oxidized Ti-Ce alloy which contained 0.7% Ce after being creep tested to fracture for 396 hours at 538° C. and a stress of 5000 p.s.i.

One aspect of the invention comprises forming an alloy of titanium with an amount of a rare earth metal ranging up to its solid solution maximum in the titanium alloy.

15 In the case of cerium or lanthanum (note FIGS. 1 and 2), the amount may range up to about 5% by weight. The binaries of FIGS. 1 and 2 are derived from the work of E. N. Savitskii and G. C. Burkanov ("Phase Diagrams for the Systems Titanium-Lanthanum and Titanium-Cerium"; Academie of Science Journal of Inorganic Chemistry, vol. 2, No. 11, 1957, page 2609). It is appreciated that these binaries may be subject to refinement through additional investigation and, therefore, the maximum of 5% given above could vary one way or the other. In 20 any event, so long as the amount of rare earth metal employed ranges up to its equilibrium maximum in the solid solution, the results of the invention will be achieved.

25 I prefer that the amount of rare earth metal employed in forming the solid solution, e.g. Ce or La, not exceed about 1% and, more preferably, range from about 0.05 to 0.8% by weight.

30 35 I then fabricate the alloy after which it is subjected to heat treatment at an elevated temperature in an oxygen-containing environment to effect absorption of oxygen by solution sufficient to convert substantially all of the rare earth metal to finely dispersed rare earth metal oxide of high melting point.

40 45 I have found cerium to be preferably suitable as the solute element in carrying out my invention. It, like the other rare earth metals, has a higher free energy of formation of the oxide ( $\text{CeO}_2$ ) per gram atom of oxygen than the heat of solution of oxygen in the solvent metal titanium and therefore can be selectively oxidized in the presence of titanium. Oxygen has a very low solubility in cerium: in addition, the oxide of cerium is substantially insoluble in titanium at fabrication and application temperatures, and furthermore is a very stable refractory oxide under operating condition.

50 55 In one specific embodiment of the invention, after the Ti-Ce alloy has been worked into the desired shape, the alloy is heated to a temperature at which the alpha phase prevails for the particular amount of rare earth metal employed, for example within the range of about 650 to 875° C., to insure substantially complete solution of the cerium in alpha titanium, after which the thus-heated alloy is then subjected to internal oxidation at a temperature ranging up to about 875° C., preferably within the alpha region, e.g. from about 650° C. to 875° C., under controlled oxidizing conditions adapted to prevent the 60 build up of an oxygen concentration gradient of an oxygen barrier. In other words, the conditions are such as to maintain a slow rate of oxygen solution into the titanium. This may be accomplished by using a system in which oxygen has a pressure ranging from about 0.1 to 200 microns. One means of accomplishing this is to carry out the oxidizing treatment in a vacuum system having a known leak rate of air, for example a leak rate adapted to maintain a vacuum ranging from about 0.5 micron to 200 microns, preferably from about 0.5 micron to 50 microns. Or the oxidizing treatment may be carried out in a low pressure oxygen atmosphere diluted with an inert

gas, e.g. argon, in which the oxygen partial pressure is between about 0.1 and 20 microns.

Another specific embodiment for converting the cerium, or other rare earth metal, to a substantially uniformly dispersed phase of cerium oxide comprises subjecting the wrought Ti-Ce alloy to heating at a temperature within the alpha region of the Ti-Ce binary, e.g. the temperature range of about 650° C. to 875° C. to insure solid solution of cerium in the alpha titanium followed by quenching to retain the solid solution. The alloy is then reheated to a temperature in the alpha plus cerium region, for example over the temperature range of about 400° C. to 650° C. to precipitate cerium as finely dispersed particles followed by internal oxidation at a temperature within the alpha plus cerium region, e.g. 400° C. to 650° C. One advantage of having cerium so precipitated throughout the alpha matrix prior to oxidation is that control of the particle size, shape and distribution is achieved to yield more reproducible properties. Another advantage resides in the fact that lower internal 20 oxidation temperatures can be utilized.

As illustrative of the invention, the following example is given:

High purity titanium sponge containing 0.071% O<sub>2</sub>, 0.007% N<sub>2</sub>, 0.0013% H<sub>2</sub>, 0.062% Fe and 0.031% C was 25 charged into a tungsten arc furnace under a positive pressure of argon. Each amount of charge was sufficient to form a 100 gram casting. Cerium of 99.9 plus purity was employed in forming two charges, one containing 0.2% and the other 0.7%. In order to minimize oxide pick up as much as possible, each of the cerium additions in the form of cubes were carefully cleaned of surface oxides by polishing on all sides with fine silicon carbide powder just prior to melting to minimize the addition of cerium as cerium oxide.

Each of the castings obtained was subjected to cold working by cold press forging to 50% reduction in area and then were cold rolled to 0.01 inch thickness, using a series of 14 passes with no intermediate anneal between passes. The rolled strips were sheared into pieces one 40 inch wide by four inches long. To recrystallize and solutionize any cerium which might be out of solution, the pieces were stacked in groups of 20, with a strip of pure molybdenum between each piece to prevent welding during heating, clamped between two heavy plates of titanium, and heated at 850° C. for two hours in a vacuum of 0.25 micron. The pieces were quenched from 850° C. to a temperature below 300° C. by flushing purified helium through the vacuum chamber at a rate of 200 cubic feet per hour.

The recrystallized pieces were then subjected to internal oxidation by suspending them in a vacuum furnace by fine titanium wire and heating to 850° C. at a leak rate of air to maintain a vacuum of ten microns. The strips containing 0.2% Ce were held at temperature for two hours while those which contained 0.7% Ce were held for four hours. All specimens were furnace cooled under vacuum.

In determining the extent to which the cerium had been oxidized, samples were taken from each alloy group and brominated at 200° C. At this temperature, titanium reacts with bromine vapor to form TiBr<sub>4</sub> gas which can be flushed from the system by passage of helium. The residue of this reaction contains all the unreacted compounds plus any non-volatile bromides. Thus, CeO<sub>2</sub> particles in the alloy would remain as CeO<sub>2</sub> and any elemental cerium in the alloy would convert to CeBr<sub>3</sub>, which would also remain in the residue. Titanium can never be completely removed by bromination at this temperature. Since dissolved oxygen is not removed, titanium will be removed only as long as it is in excess of the 70 amount necessary to form TiO<sub>2</sub>.

X-ray patterns from the bromine residue of the two alloys showed lines for TiO<sub>2</sub> and CeO<sub>2</sub> only. There were no lines for CeBr<sub>3</sub>, indicating the virtual absence of elemental cerium in the structure. In other words, substan-

tially all of the cerium was converted to CeO<sub>2</sub> by internal oxidation.

Stress-rupture specimens 4 inches x 1 inch with a 2 inch gage length and a 0.354 inch gage width, meeting 5 ASTM requirements, were stamped out of the 4 inches x 1 inch strips by means of a punch and die. Specimens were tested on standard creep rupture frames. Due to the thickness of the strips, actual loads were small and direct bottom loading was used rather than beam loading. Specimens were tested at these temperatures: 426, 538 and 648° C. (800, 1000 and 1200° F.); and at stresses selected to yield rupture life values of less than one to 300 hours and above. Control tests were also run on the unalloyed titanium melted in the same furnace and worked in the same manner.

The results of the stress rupture tests obtained on the unalloyed titanium and the Ti-Ce compositions are given in Tables I, II and III as follows:

TABLE I  
Titanium

| Stress in p.s.i. | Temperature, °C. | Life in Hours | Percent Elongation |
|------------------|------------------|---------------|--------------------|
| 14,000           | 426              | .0011         | -----              |
| 12,000           | 426              | .067          | 10.2               |
| 11,000           | 426              | 2.000         | 16.0               |
| 10,000           | 426              | 61.883        | 21.9               |
| 6,000            | 426              | 122.00        | 44.5               |
| 8,000            | 648              | 0.325         | 14.2               |
| 6,000            | 648              | .0680         | 34.4               |
| 4,000            | 648              | .348          | 45.7               |
| 2,000            | 648              | 3.57          | 53.6               |
| 1,000            | 648              | 40.08         | 12.4               |

TABLE II  
Titanium with 0.2% Ce (Internally Oxidized)

| Stress in p.s.i. | Temperature, °C. | Life in Hours | Percent Elongation |
|------------------|------------------|---------------|--------------------|
| 18,000           | 426              | .050          | 9.3                |
| 16,000           | 426              | .191          | 19.8               |
| 14,000           | 426              | 4.133         | 30.8               |
| 12,000           | 426              | 40.00         | 42.1               |
| 10,000           | 426              | 480.20        | 57.9               |
| 13,000           | 538              | .030          | 38.2               |
| 45 12,000        | 538              | .678          | 41.4               |
| 10,000           | 538              | 2.583         | 47.3               |
| 8,000            | 538              | 9.23          | 53.1               |
| 5,000            | 538              | 90.45         | 62.8               |
| 8,000            | 648              | .0636         | 31.3               |
| 6,000            | 648              | .517          | 50.1               |
| 4,000            | 648              | .8.26         | 68.7               |
| 3,000            | 648              | 72.21         | 30.5               |
| 2,000            | 648              | 629.45        | 20.7               |

TABLE III  
Titanium with 0.7% Ce (Internally Oxidized)

| Stress in p.s.i. | Temperature, °C. | Life in Hours | Percent Elongation |
|------------------|------------------|---------------|--------------------|
| 18,000           | 426              | .0167         | 15.00              |
| 16,000           | 426              | .71           | 26.2               |
| 14,000           | 426              | 44.90         | 37.5               |
| 13,000           | 426              | 661.2         | 45.4               |
| 12,000           | 426              | 480.33        | 48.6               |
| 14,000           | 538              | .0206         | 27.1               |
| 12,000           | 538              | .484          | 36.3               |
| 10,000           | 538              | 1.75          | 46.0               |
| 8,000            | 538              | 10.09         | 55.2               |
| 6,000            | 538              | 104.15        | 64.2               |
| 5,000            | 538              | 396.02        | 66.7               |
| 9,000            | 648              | .0398         | 31.6               |
| 8,000            | 648              | .224          | 40.5               |
| 6,000            | 648              | 1.616         | 57.5               |
| 5,000            | 648              | .8.20         | 67.0               |
| 4,000            | 648              | 43.85         | 41.0               |
| 3,000            | 648              | 237.30        | 32.2               |

A log-log plot of stress against rupture life showed flat curves indicative of stability at elevated temperatures.

In general, the oxidized titanium-cerium alloys are markedly superior to pure titanium at all stresses and tem-

peratures as is evident from the following correlation of Table IV:

TABLE IV

| Material        | Stress,<br>p.s.i. | Temp.,<br>° C. | Life in<br>Hours |
|-----------------|-------------------|----------------|------------------|
| Titanium.....   | 12,000            | 426            | 0.067            |
| Ti-0.2% Ce..... | 12,000            | 426            | 40.00            |
| Ti-0.7% Ce..... | 12,000            | 426            | 480.33           |
| Titanium.....   | 10,000            | 426            | 61.9             |
| Ti-0.2% Ce..... | 10,000            | 426            | 480.2            |
| Titanium.....   | 4,000             | 648            | 0.348            |
| Ti-0.2% Ce..... | 4,000             | 648            | 8.26             |
| Ti-0.7% Ce..... | 4,000             | 648            | 43.85            |
| Titanium.....   | 3,000             | 648            | 11.1             |
| Ti-0.2% Ce..... | 3,000             | 648            | 72.21            |
| Ti-0.7% Ce..... | 3,000             | 648            | 287.30           |

<sup>1</sup> Extrapolated.

The microstructures of the internally-oxidized alloys were composed of equiaxed alpha grains with a dispersion of fine phase particles within the grains and at grain boundaries. The dispersion, although concentrated somewhat preferentially at grain boundaries, appears to be well distributed as shown in FIG. 3. Furthermore, there is no particle size gradient across the specimen. The appearance of some coarse particles was noted which was believed to be due to the introduction of some cerium as CeO<sub>2</sub> into the melt on the surface of the cerium charge.

The microstructure after testing at these temperatures consists of recrystallized alpha grains characterized by irregular grain boundaries and a sub-structure within the grains. A point of interest in these microstructures was the distribution of the dispersed phase, which no longer exists primarily at grain boundaries but rather is found clustered in lines or groups running through grains and across boundaries. FIG. 4 is typical of this type of structure. Note that the grain size is still very fine. The fact that the particles have not coalesced after long times at temperatures shows the stability of CeO<sub>2</sub> in titanium and the absence of elemental cerium in the structure.

The results of the internal oxidation of cerium in titanium indicate that significant benefits in the strength of titanium can be achieved for service up to at least 1200° F. Lower oxidation temperatures are indicated to produce more of the much finer CeO<sub>2</sub> particles and smaller interparticle spacing for optimum high strength properties.

In order to optimize the strengthening obtained by dispersion hardening through internal oxidation, it is preferred that the thickness of the titanium material being treated not exceed about 0.25 inch, whether the material be in the form of particles, strip, sheet, rods, etc. Larger sizes can be internally oxidized depending upon the amount of time employed.

Where the material is desired for the powder metallurgy production of titanium articles, the wrought alloy is comminuted below  $\frac{1}{4}$  inch in size and preferably comminuted to yield particles ranging in size from about 10 mesh down to 100 mesh or lower followed by internal oxidation as described herein. The internally oxidized powder is then consolidated and followed by sintering and/or extrusion to the desired shape.

The advantage of the powder metallurgy method of production is that it enables the production of thick shapes in excess of one quarter inch section having a uniform dispersion throughout of the rare earth metal oxide. This is because each particle already contains a random dispersion of the oxide achieved through internal oxidation. In utilizing the powder metallurgy technique, the internally oxidized comminuted material is consolidated by pressure into a slug of green strength at least about 60 to 80% of true density and the slug sintered if necessary in a non-reactive environment to further strengthen it. The slug is then subjected to hot working, such as by hot extrusion, by encasing it in a metal sheath, such as iron or nickel, and the whole reduced in size at an extrusion ratio of at least 15 to 1, and preferably from about 20 to 1 to

25 to 1, with extrusion pressures ranging up to 250 tons per square inch for temperatures ranging from about 950° C. to 1350° C., the amount of extrusion pressure employed depending on the temperature used. After completion of the working, the sheath metal is removed by pickling, grinding or other means. Thus, large sized rounds can be produced or rectangular shapes, angles and other contours while at the same time being dispersion hardened throughout.

10 While the invention has been described with respect to improving the strength properties of titanium metal, it is also applicable to the strengthening of titanium alloys containing at least 80% titanium. Examples of such alloys include 10 to 20% molybdenum and the balance titanium, 8% manganese and the balance titanium, titanium containing 2% copper, and a Ti-Si alloy containing 2% silicon, and others. The expressions "titanium-base alloys" or "titanium substantially the balance" are meant to cover such composition as well as titanium itself.

15 Because of the chemical and metallurgical similarities between titanium and zirconium, the invention is also applicable to zirconium and likewise to hafnium, both of which fall in the titanium metal group. The invention also includes alloys based on these metals, that is alloys containing at least 80% of one or more of the titanium group metals Ti, Zr and Hf.

20 Examples of other rare earth metals which may also be employed in carrying out the invention besides Ce and La are Pr, Nd, II, Sm, Eu, Gd, etc. Of these 30 gadolinium and lanthanum are particularly attractive along with cerium. Thorium likewise may be employed. Depending on the extent to which these elements go into solid solution with titanium or titanium-base alloys, alloys containing these elements may be similarly treated 25 as the cerium-containing titanium alloy described hereinbefore.

25 Although the present invention has been described in conjunction with preferred embodiments, it is to be understood that modifications and variations may be resorted to without departing from the spirit and scope of the invention, as those skilled in the art will readily understand, and such modifications and variations are considered to be within the purview and scope of the invention and the appended claims.

30 What is claimed is:

1. A method of dispersion hardening a matrix metal comprising essentially at least about 80% of at least one element selected from the group consisting of Ti, Zr and Hf, said matrix metal being characterized by an alpha to beta transformation temperature which comprises, forming an alloy of said matrix metal and cerium with up to about 5% of cerium but not exceeding the maximum solubility of said cerium in the alpha solid solution of the matrix metal, and then subjecting said alloy to internal oxidation at an elevated temperature not exceeding the temperature at which the alpha phase transforms to beta in an oxidizing atmosphere corresponding to an oxygen pressure not exceeding the amount at which oxygen build up occurs as an oxygen gradient at 35 the alloy interface, whereby to promote a controlled rate of oxygen diffusion into said alloy and convert selectively substantially said contained cerium to refractory metal oxide finely dispersed throughout the matrix metal.

2. A method of dispersion hardening a matrix metal comprising essentially at least about 80% titanium, said matrix metal being characterized by an alpha to beta transformation temperature which comprises, forming an alloy of said matrix metal and cerium with up to about 5% cerium but not exceeding the maximum solubility 40 of said cerium in the alpha solid solution of the matrix metal, and then subjecting said alloy to internal oxidation at an elevated temperature not exceeding the temperature at which alpha phase transforms to beta in an oxidizing atmosphere corresponding to an oxygen pressure not exceeding the amount at which oxygen build up occurs

as an oxygen gradient at the alloy interface, whereby to promote a controlled rate of oxygen diffusion into said alloy and convert selectively substantially said contained cerium to refractory metal oxide finely dispersed throughout the matrix metal.

3. The method of claim 2, wherein said matrix metal is comprised essentially of titanium, wherein cerium ranges up to about 1% by weight, and wherein prior to internal oxidation the alloy is formed into a shape having a thickness of up to about 0.25 inch and is heated to an elevated temperature to effect solution of said cerium in the alpha solid solution of the alloy.

4. The method of claim 2, wherein the amount of cerium ranges from about 0.05 to 0.8% by weight, wherein prior to oxidation the alloy shape is heated to an elevated temperature ranging from amount 650° C. to 875° C. within the alpha solid solution of the alloy to effect solution of the cerium in the solid solution, and wherein the internal oxidation following thereafter is conducted at an elevated temperature not exceeding about 875° C.

5. The method of claim 4, wherein after the alloy is heated to the temperature within the alpha solid solution region it is quenched to retain said solid solution followed by heating the alloy to a temperature outside said alpha solid solution to effect precipitation of finely divided cerium particles prior to subjecting the alloy to internal oxidation.

6. The method of claim 5, wherein the temperature for precipitating finely divided cerium particles ranges from about 400° C. to 650° C.

7. A method of dispersion hardening a matrix metal comprising essentially at least about 80% titanium, said matrix metal being characterized by an alpha to beta transformation temperature which comprises, forming an alloy of said matrix metal and cerium with up to about 5% of cerium but not exceeding the maximum solubility of said cerium in the alpha solid solution of the matrix metal, comminuting said alloy, and subjecting said comminuted alloy to internal oxidation at an elevated temperature not exceeding the temperature at which the alpha phase transforms to beta in an oxidizing atmosphere corresponding to an oxygen pressure not exceeding the amount at which oxygen build up occurs as an oxygen gradient at the alloy interface, whereby to promote a controlled rate of oxygen diffusion into said alloy and convert selectively substantially said contained cerium to refractory metal oxide finely dispersed throughout the matrix of the comminuted alloy.

8. The method of claim 7, wherein the matrix metal

is comprised essentially of titanium and wherein the amount of cerium ranges up to about 1% by weight.

9. The method of claim 8, wherein prior to internal oxidation the comminuted alloy is heated to an elevated temperature within the alpha solid solution region of the alloy, wherein the alloy is quenched to retain said solid solution, and wherein said comminuted alloy is heated to an elevated temperature outside said alpha solid solution to effect precipitation of finely divided cerium particles.

10. A dispersion hardened matrix metal comprised essentially of at least about 80% of at least one element selected from the group consisting of Ti, Zr and Hf and containing an amount of cerium metal ranging up to about 5% by weight but not exceeding the maximum solubility of said cerium in the alpha solid solution of the matrix metal, said cerium being dispersed throughout the matrix metal in the form of finely divided refractory oxide.

11. The dispersion hardened metal of claim 10, wherein the matrix metal is comprised essentially of titanium and wherein the cerium ranges up to about 1% by weight.

12. As an article of manufacture, a dispersion hardened wrought alloy product comprised essentially of titanium containing up to about 1% cerium dispersed throughout the matrix of said alloy in the form of finely divided cerium oxide.

13. The article of manufacture as defined in claim 12, wherein the cerium content ranges from about 0.05 to 0.8% by weight.

#### References Cited in the file of this patent

##### UNITED STATES PATENTS

|           |                       |               |
|-----------|-----------------------|---------------|
| 2,539,298 | Doty et al. -----     | Jan. 23, 1951 |
| 2,669,512 | Doty et al. -----     | Feb. 16, 1954 |
| 2,678,268 | Ham -----             | May 11, 1954  |
| 2,766,113 | Chisholm et al. ----- | Oct. 9, 1956  |
| 2,818,336 | Swazy et al. -----    | Dec. 31, 1957 |
| 2,823,988 | Grant -----           | Feb. 18, 1958 |
| 2,894,838 | Gregory -----         | July 14, 1959 |

##### FOREIGN PATENTS

|         |                     |              |
|---------|---------------------|--------------|
| 645,681 | Great Britain ----- | Nov. 8, 1950 |
|---------|---------------------|--------------|

##### OTHER REFERENCES

Dispersion Hardening of Sintered Titanium Alloys by Refractory Metal Powder Additions, PB 131, 937, March 5, 1958, pp. 12 and 13.

Hansen, "Constitution of Binary Alloys," copyright 1958 by McGraw-Hill, pp. 463, 893, and 1232.

UNITED STATES PATENT OFFICE  
CERTIFICATE OF CORRECTION

Patent No. 3,070,468

December 25, 1962

Nicholas J. Grant

It is hereby certified that error appears in the above numbered patent requiring correction and that the said Letters Patent should read as corrected below.

Column 7, line 13, for the claim reference numeral "2" read -- 3 --; lines 19 and 20, strike out "is conduct- in internal oxidation following thereafter".

Signed and sealed this 4th day of June 1963.

(SEAL)

Attest:

ERNEST W. SWIDER  
Attesting Officer

DAVID L. LADD  
Commissioner of Patents